

2,825,684

## BRIGHT COPPER PLATING

Christian J. Wernlund, Niagara Falls, N. Y., assignor to E. I. du Pont de Nemours and Company, Wilmington, Del., a corporation of Delaware

No Drawing. Application October 9, 1956  
Serial No. 614,825

6 Claims. (Cl. 204—52)

This invention relates to the production of bright copper electroplate from aqueous baths containing selenium as a brightening additive. It has as its principal objects provision of selenium-containing, electroplating baths of extended bright-plating ranges and of methods for plating from the baths.

The present application is a continuation-in-part of my copending application Serial Number 352,268, filed April 30, 1953, now abandoned.

Inorganic selenium compounds such as the selenites and selenates have been employed heretofore in aqueous electroplating baths. Thus Weiner, Alien Property Custodian Publication Serial Number 351,241, published May 18, 1943, shows these compounds in silver plating baths and intimates that they may be utilized in copper cyanide baths. Actual trial of selenites and selenates in the latter baths has shown that they do have some brightening characteristics.

In accordance with this invention, it has now been found that the bright plating range of aqueous copper cyanide baths carrying as a brightening agent an inorganic selenium compound, particularly an oxygen-containing selenium compound, can be extended by the simultaneous use of certain other metallic additives. These additives are cadmium, bismuth and silver.

There are numerous substantially conventional aqueous copper cyanide baths any one of which may be employed as the basic bath of the invention. Preferably they are made up from potassium salts and contain, in aqueous solution:

| Component                   | Satisfactory Range (oz./gal.) | Preferred Range (oz./gal.) |
|-----------------------------|-------------------------------|----------------------------|
| Potassium hydroxide.....    | 1-10                          | 1-8                        |
| Free potassium cyanide..... | 0.5-4                         | 1-2                        |
| Copper cyanide.....         | 5-20                          | 8-14                       |

The "free" potassium cyanide is that measured by the Liebig silver nitrate titration.

The cheaper sodium compounds may be substituted in whole or in part for those of potassium. Since the potassium formulations permit higher rates of copper deposition and produce slightly brighter deposits, they are technologically preferred.

The inorganic selenium compounds employed as brightening additives in the invention are preferably oxygen-containing compounds such as selenous and selenic oxides and acids and the corresponding salts, e. g., sodium and potassium selenite and selenate. The compound utilized must, of course, be soluble to some extent in the bath and should introduce no interfering or deleterious ion.

The quantity of selenium added is not sharply critical and may vary within limits. Thus about 0.612-6.12 g./l. of additive considered as metallic selenium is usable with about 0.612-3.00 g./l. preferred. The weight of compound chosen should yield this weight of metal, the cor-

responding weight of  $H_2SeO_3$ , selenous acid, for example, being about 1-10 g./l.

The form of the additive employed with the selenium is also not particularly critical. Thus about any compound form of the additive may be used that is compatible with the bath, i. e., is soluble in the bath and does not change important bath characteristics such as pH. Cadmium and silver are generally added as the cyanides,  $Cd(CN)_2$  and  $Ag(CN)$ . Complex cyanides such as  $KAg(CN)_2$  and other compounds are also usable. Trivalent bismuth compounds such as  $Bi(C_6H_9O_6)_3 \cdot 7H_2O$  represent the form preferred for this metal.

The quantity of the second metal added varies to some extent with the metal. It is generally rather small, but variable within limits. Usable ranges are, for cadmium, about 0.007-7.0 g./l., for bismuth, about 0.002-0.05 g./l. and, for silver, about 0.008-1.62 g./l. Preferred ranges are 0.070-3.50, 0.002-0.01, and 0.008-0.08 g./l., respectively. Typical compound weights are 0.01-10 g./l. for  $Cd(CN)_2$ , 0.01-0.2 g./l. for  $Bi(C_6H_9O_6)_3 \cdot 7H_2O$ , and 0.01-2.0 for  $AgCN$ .

Each of the three metallic additives used simultaneously with selenium has some brightening characteristics of its own within narrow current density ranges. The effects produced by the respective combinations are, however, much greater than the separate effects. The combined additives may, therefore, properly be called synergistic in their application.

It will be understood that not all metals are synergistically cooperative with selenium in cyanide copper baths. Thus such elements as zinc, arsenic, cobalt and iron do not effect any improvements in the plating or the deposit when employed with selenium.

The baths of this invention may produce rough deposits unless precautions are taken thereagainst. Known anti-pitting agents are, therefore, preferably added to the bath. Agents like betaines, e. g., C-decyl betaine shown by the Holt U. S. Patent 2,255,057, are satisfactory. A preferred agent contains about 30% of trimethyl benzyl ammonium chloride and 12.5% of C-decyl betaine, the remainder being water, and is supplied to the extent of about 5 g./l. of bath.

The conditions necessary for plating from the baths of this invention are substantially those of conventional aqueous copper cyanide plating. Thus the temperature may vary between about 60 and 95° C. with about 80° C. preferred. Agitation as by stirring may be used if desired. Choice of the material of the cathodes or workpieces is optional.

A particular advantage of this invention is that it produces bright copper plate over a wider range of current densities (amperes/ft.<sup>2</sup>—a./s. f.) or, in some instances, brighter copper than a copper cyanide bath containing no additive or any one of the four metallic additives alone. In some embodiments, bright plate may be formed continuously in a range of about 10-60 a./s. f. or even more. The plating of irregular objects having projections and recesses is consequently greatly simplified.

There follow some examples intended to illustrate, but not to limit, the invention in more detail. In these examples all percentages are by weight.

## Example I

This example shows the effect of selenium and cadmium as joint plating additives.

(a) There was made up a conventional aqueous copper cyanide electroplating solution containing 14 oz./gal. of cuprous cyanide, 2.0 oz./gal. of free sodium cyanide, 6.0 oz./gal. of potassium hydroxide and 1.5 oz./gal. of sodium carbonate. 5 g./l. of the preferred C-betaine anti-pitting compound noted above were also added.

This conventional solution was placed in a 1000 ml.

oscillating cathode Hull cell at a temperature of  $80^{\circ} \pm 2^{\circ}$  C. and a test run made to determine the bright plating range. No bright plate was obtained at a current density above about 10 a./s. f.

(b) To a portion of the conventional bath of (a) was added 0.2 g./l. of  $\text{Cd}(\text{CN})_2$  and plating carried out as in (a). A bright plating range of 35-52 a./s. f. was obtained.

A control run with 1.0 g./l. in the bath and in the manner of (a) gave a very bright plating range of 16-37 a./s. f. with a hazy band at about 22-25 a./s. f. This hazy band is very undesirable since it occurs about in the center of the bright plating range of selenium alone.

Part of the bath of (a) containing both 0.2 g./l. of  $\text{Cd}(\text{CN})_2$  and 1 g./l. of selenous acid showed a single very bright plating range from 13 to 36 a./s. f. with no hazy band.

#### Example 2

This example shows the use of selenium and silver as joint plating additives.

The basic sodium cyanide bath of I (a) gave a very bright plating range of 12-35 a./s. f. when containing 1.0 g./l. of silver cyanide and 2.0 g./l. of selenous acid. The silver cyanide alone gave bright plating ranges of 10-20 and 35-60 a./s. f. while 2 g./l. of selenous acid gave about the same results as 1 g./l. of the same material, i. e., a very bright range of 13-36 a./s. f. with an extremely undesirable hazy band at 22-25 a./s. f.

#### Example 3

This example shows the use of selenium and bismuth as joint additives.

A potassium-based plating bath was formulated containing about 14 oz./gal. of cuprous cyanide, 1 oz./gal. of free potassium cyanide, 5 oz./gal. of potassium hydroxide and 0.67 oz./gal. of the aqueous anti-pitting agent containing about 30% of trimethyl benzyl ammonium chloride and 12.5% of C-decyl betaine. When tested in a Hull cell, this bath alone gave no bright plate above 10 a./s. f.

When 0.030 g./l. of bismuth trioxide and 2.0 g./l. of selenous acid were employed together in the potassium-containing bath, bright plate was obtained in the ranges 10-20 and 26-60 a./s. f. Hazy, streaked plate was ob-

tained in the range 21-26 a./s. f. The bismuth when used alone produced bright plate only in the 9-20 a./s. f. range. The selenium produced no bright plate above 30 a./s. f.

The embodiments of the invention in which an exclusive property or privilege is claimed are defined as follows:

1. An aqueous bath for electrodepositing bright copper containing copper cyanide and a dual metallic brightening agent comprising about 0.612-6.12 g./l. of metallic selenium supplied as a member of the group consisting of the selenium oxides, selenous and selenic acids and the alkali metal salts of said acids, and a soluble compound of a metal taken from the class consisting of cadmium in an amount from about 0.007 to 7 g./l., bismuth in an amount from about 0.002 to 0.05 g./l., and silver in an amount from about 0.008 to 1.62 g./l.

2. An aqueous bath for electrodepositing bright copper containing copper cyanide, about 0.612-3.00 g./l. of selenium supplied as a member of the group consisting of the selenium oxides, selenous and selenic acids and the alkali metal salts of said acids, and 0.070-3.50 g./l. of dissolved cadmium.

3. An aqueous bath for electrodepositing bright copper containing copper cyanide, about 0.612-3.00 g./l. of selenium supplied as a member of the group consisting of the selenium oxides, selenous and selenic acids and the alkali metal salts of said acids, and 0.002-0.01 g./l. of dissolved bismuth.

4. An aqueous bath for electrodepositing bright copper containing copper cyanide, about 0.612-3.00 g./l. of selenium supplied as a member of the group consisting of the selenium oxides, selenous and selenic acids and the alkali metal salts of said acids, and 0.008-0.08 g./l. of dissolved silver.

5. The bath of claim 1 containing additionally an anti-pitting agent.

6. The bath of claim 5 in which the anti-pitting agent is a betaine.

#### References Cited in the file of this patent

#### UNITED STATES PATENTS

|           |                 |               |
|-----------|-----------------|---------------|
| 2,732,336 | Ostrow          | Jan. 24, 1956 |
| 2,737,485 | Overcash et al. | Mar. 6, 1956  |
| 2,770,587 | Ostrow          | Nov. 13, 1956 |